

## UNITED STATES PATENT OFFICE

1,935,213

## SURFACE ORNAMENTATION

Leo J. Mitchell, St. Louis, Mo.

No Drawing. Application August 24, 1931  
Serial No. 559,133

6 Claims. (Cl. 91—70)

My invention relates to the ornamentation of surfaces, particularly wood and metal surfaces, and it has for its principal object to provide a surface ornamentation that is highly durable and of beautiful appearance, having a highly lustrous finish such as is produced by metal plating. The invention consists principally in the ornamenting of surfaces by applying thereto a thin coat of a compound of bismuth and baking the article to make said coat permanent. The invention further consists in the process of surface ornamentation hereinafter described and claimed.

A satisfactory preliminary treatment for my process is to apply to the surface, preferably by a spray gun, a suitable coating comprising varnish base, bronzing liquid, lacquer or the like having mixed therewith any of the well known metal powders, (such as bronze, silver, aluminum and gold bronze) followed by a coating of clear varnish. This preliminary coating may be permitted to dry in air or the article may be baked. The preliminary coatings commonly used may be baked at a temperature of about 180° F. for ten minutes.

25 After the preliminary coating has hardened, my process comprises applying over said first coating a thin coating of finely divided bismuth or of a powdered bismuth compound. Bismuth oxychloride is especially suitable for the purpose. 30 The bismuth compound may be applied in a thin even layer by rubbing it on with cotton, chamois, or other suitable soft material. The bismuth coating, after a slight rubbing, assumes a highly polished and lustrous appearance similar to that of metal plate.

Under some conditions, no further treatment may be required after the application of the bismuth; but in order to make the finish permanent on articles that are to be handled, I bake 40 the article sufficiently to soften the preliminary coat and enable the bismuth coat to adhere firmly thereto. Excessive temperature should be avoided. In the case of a preliminary coat having a synthetic resin base, a temperature of about 180° F. and a baking of not to exceed two hours are satisfactory. This baking operation makes the finish permanent, but without injuring its lustrous appearance.

50 Any desired color scheme may be obtained by suitable changes in the materials used in the preliminary coating and also the particular bismuth compound used. The process is applicable to the ornamentation of the surface of any article that will withstand the baking operation. It

is particularly applicable to metal and wood articles.

What I claim is:

1. The process of surface ornamentation which comprises applying to the surface of an article 60 a preliminary coating of a metallic powder mixed with a suitable resinous base material, hardening said preliminary coating, applying thereto a compound of bismuth in a thin layer and baking the article sufficiently to soften the base material of 65 said preliminary coating.

2. The process of ornamenting metal surfaces coated with a substance having a resinous base, which comprises applying over said coating, a halogen salt of bismuth in a thin layer and then 70 baking the article.

3. The process of ornamenting metal surfaces coated with a substance having a resinous base, which comprises applying over said coating, a halogen salt of bismuth in a thin layer and then 75 baking the article at a temperature of about 180° Farenheit.

4. The process of ornamenting metal surfaces coated with a substance having a resinous base, which comprises applying over said coating, bismuth oxychloride in a thin layer and then 80 baking the article.

5. The process of ornamenting metal surfaces coated with a substance having a resinous base, which comprises applying over said coating, bismuth oxychloride in a thin layer and then 85 baking the article at a temperature of about 180° Farenheit.

6. The process of surface ornamentation which comprises applying to the surface of an article a 90 preliminary coating of a metallic powder mixed with a suitable resinous base material, hardening said preliminary coating, applying thereto bismuth oxychloride in a thin layer and then baking the article sufficiently to soften the base material of 95 said preliminary coating.

LEO J. MITCHELL.

100

105

110